

## UNITED STATES PATENT OFFICE

2,156,918

## STABILIZED SOLUTIONS OF METAL-ORGANIC COMPOUNDS AND METHOD OF MAKING THE SAME

Willard E. Lyons, Chicago, Ill., assignor to Leo Corporation, Chicago, Ill., a corporation of Illinois

No Drawing. Application May 7, 1937,  
Serial No. 141,255

## 12 Claims. (Cl. 44-9)

This invention relates to stabilized solutions of metal-organic compounds and to a method of making the same. More particularly the invention relates to the stabilization of motor fuels comprising liquid hydrocarbons containing dissolved metal organic compounds, by the addition thereto of acid reacting substances soluble in water but relatively insoluble in the liquid hydrocarbons.

10 Metal organic compounds, for instance the heavy metal compounds of beta diketones, are susceptible to hydration or hydrolysis when water is present. This is true when such compounds are dissolved in liquid hydrocarbons, such as gasoline and the like, as in the manufacture of anti-knock motor fuels, for the reason that minor proportions of water are almost invariably associated with the liquid hydrocarbons. Water, for example, finds its way into receptacles containing motor fuels by virtue of the breathing action that takes place, the moisture introduced with the air into the receptacle being condensed quite largely around the walls and accumulating at the bottom of the receptacle. Also, due to the very slight solubility of water in gasoline, a very minor proportion of water may be dispersed in the body of gasoline delivered for use as the motor fuel.

I have now found that the tendency of metallic compounds to become hydrolyzed or hydrated, 30 due to the presence of water in motor fuels or in the receptacles in which the motor fuels are stored, may be inhibited by the addition to the water phase of an acid reacting substance capable of furnishing a sufficient hydrogen ion concentration to retard or even prevent such action from taking place. In the absence of such inhibiting action, the water present would tend to cause hydrolysis or hydration of the metal organic compounds with the formation of basic salts or bases 40 of the metal which are insoluble both in the motor fuel and in the water present. The addition to the water, however, of acid reactive substances in accordance with this invention prevents such precipitation of metal bearing substances over a 45 substantial period of time.

It is therefore an important object of this invention to provide a method of stabilizing solutions of metal organic compounds in liquid hydrocarbons where water is present or is likely to 50 become associated with the liquid hydrocarbons.

It is a further important object of this invention to provide a method of stabilizing motor fuels having dissolved therein compounds of beta diketones with heavy metals where such compounds 55 are susceptible to hydrolysis or hydration in the presence of water.

It is a further important object of this invention to provide a stabilized solution of heavy metal compounds of beta diketones in liquid hydrocarbons, such as motor fuels and the like,

wherein the stabilizing agent is an acid reacting substance soluble in water but relatively insoluble in the liquid hydrocarbons.

Other and further important objects of this invention will become apparent from the following description and appended claims.

The liquid hydrocarbons to which my invention is particularly directed are those generally employed as motor fuels, such as gasoline, benzene, polymerized hydrocarbons, or blends thereof. Of the metal organic compounds which may be added to such hydrocarbons for increasing the efficiency of their combustion in internal combustion engines, the heavy metal compounds of the beta diketones have been found particularly useful. The metals intended to be included by the term "heavy metals" are those classified in the periodic table shown in Demings General Chemistry, fourth edition. These compounds, while forming relatively stable solutions in liquid hydrocarbons that are free from water, have a tendency to form insoluble precipitates when water is present, due probably to hydrolysis or hydration with the consequent formation of basic salts of the compounds or bases of the metal.

In accordance with the method of this invention, an acid reacting substance, which is water soluble but relatively insoluble in liquid hydrocarbons, is added to the solution of the heavy metal organic compounds in the liquid hydrocarbons. 30 Various acid reacting substances can be used for this purpose, such as boric acid, phosphoric acid, water soluble acid metal salts like sodium bisulfate, water soluble organic acids, such as acetic, citric, salicylic, propionic, hydroxy propionic, lactic, saccharic, formic, malic, malonic, maleic, tauric, succinic and various acidic compounds which can form water soluble salts.

If the acid reacting substance to be added to the liquid hydrocarbons solution is relatively insoluble in the hydrocarbons and has a specific gravity greater than that of the hydrocarbons, the acid reacting substance, when added to a tank or other receptacle containing the hydrocarbons, will sink to the bottom by gravity and will accumulate there in any water that may be present or that may subsequently form and collect in the bottom. In this manner, large storage tanks, tank cars and other receptacles for liquid hydrocarbons may have their contents protected 50 against the hydrolyzing or hydrating action of any water that may then be present at the time of treatment or that may subsequently accumulate during the storage period.

The amount of inhibitor to be added to any given mass of liquid hydrocarbons, gasoline or the like, will depend upon the amount of water present in association with the hydrocarbons, or the amount of water that may reasonably be expected to collect during the storage period.

In general, it is sufficient if the acid reacting substance is added to the receptacle containing liquid hydrocarbons in an amount capable of furnishing a pH numerically less than that at which the heavy metal organic compound tends to begin to form an insoluble precipitate. Since an excess of the inhibitor is not of itself harmful, unless carried over mechanically with the liquid hydrocarbons, no particular care need be taken in guarding against the use of an excess of the inhibitor.

The following examples will serve to illustrate preferred embodiments of this invention as applied to the treatment of motor fuels containing heavy metal compounds of beta diketones:

*Example No. 1*

Gasoline treated with a heavy metal beta diketone in an amount of from 0.0001% by weight 20 and upwards is contained within a large storage tank. The amount of water present in the bottom is estimated at 10 lbs. Sufficient dry boric acid is added through the top of the tank to form a saturated boric acid solution with the 25 estimated amount of water and leave an excess of boric acid for any water that may later accumulate during the expected continued length of storage of the gasoline. About 0.5 lb. of boric acid might thus be added, but as little as 0.1 lb. 30 would be immediately sufficient. The pH of the resulting boric acid solution is in the neighborhood of 5.6, which is sufficient to inhibit or prevent the hydrolysis or hydration of the heavy metal beta diketone present in the gasoline.

35

*Example No. 2*

With the same conditions as recited in Example No. 1, in place of boric acid, about  $\frac{1}{2}$  lb. of ortho-phosphoric acid is added. Being of 40 greater density, the phosphoric acid settles through the body of the gasoline and dissolves in the water present at the bottom of the tank.

*Example No. 3*

45 With the same conditions as specified in Example No. 1, in place of boric acid, about 2 lbs. of lactic acid are added.

Other acids or acid reacting substances may be similarly used in amounts sufficient to produce a water solution having a pH equal to or 50 numerically less than about 5.6.

In the foregoing examples, the heavy metal beta diketone compounds may be the acetylacetones, propionyacetones, or mixtures thereof, 55 of any one or more of the following heavy metals:

|            |                                        |
|------------|----------------------------------------|
| Cobalt     | Zirconium                              |
| Nickel     | Beryllium                              |
| Iron       | Platinum                               |
| Manganese  | Palladium                              |
| Copper     | Thorium                                |
| Lead       | Chromium                               |
| Uranium    | Aluminum                               |
| Molybdenum | Rare earth metals such as cerium, etc. |
| Vanadium   |                                        |

It will be understood, however, that other organic compounds of any of the heavy metals, which are soluble in liquid hydrocarbons and 70 which have a tendency to hydrolyze or become hydrated in the presence of water may be present instead of, or in admixture with, a beta diketone compound, and that the liquid hydrocarbon solutions thereof may be stabilized in the 75 manner hereinabove described.

In general, the organic part of the compound requiring stabilization, may be any organic acid or compound reacting as an acid to combine with a metal. Examples of such organic acids or acid reacting organic compounds are:

|                                                                                                   |    |
|---------------------------------------------------------------------------------------------------|----|
| Naphthenic and paraffinic acids                                                                   | 10 |
| Mono alkyl esters of salicylic, phthalic, camphoric, malonic and other dicarboxylic organic acids |    |
| Cresylic acid and other phenols                                                                   | 10 |
| Mercaptans                                                                                        |    |
| Aceto acetic acid esters and their homologues                                                     |    |
| Long chain saturated and unsaturated fatty acids                                                  |    |
| Aryl carboxylic acids                                                                             | 15 |

I am aware that numerous details of the process may be varied through a wide range without departing from the principles of this invention, and I, therefore, do not purpose limiting the patent granted hereon otherwise than necessitated by the prior art.

I claim as my invention:

1. The method of stabilizing a solution of a metal beta diketone in gasoline in the presence 25 of a water phase, which comprises incorporating a gasoline insoluble, but water soluble substance into said water phase to furnish hydrogen ions in an amount sufficient to inhibit the hydrolysis and hydration of said metal beta diketone compound. 30

2. The method of stabilizing a solution of a metal beta diketone in gasoline in the presence of a water phase, which comprises incorporating boric acid into said water phase to furnish hydrogen ions in an amount sufficient to inhibit the hydrolysis and hydration of said metal beta diketone compound. 35

3. The method of stabilizing a solution of a beta diketone compound of a heavy metal in 40 liquid hydrocarbons in the presence of a water phase, which comprises incorporating a gasoline insoluble, but water soluble substance into said water phase to furnish hydrogen ions in an amount sufficient to inhibit the hydrolysis and 45 hydration of said metal beta diketone compound.

4. The method of stabilizing a solution of a beta diketone compound of a heavy metal in a hydrocarbon motor fuel when in the presence of a water phase, which comprises dissolving in said 50 water phase an acid reacting compound which is relatively insoluble in the motor fuel and which in water solution provides a pH value which is numerically less than 5.6.

5. The method of stabilizing a solution of a 55 beta diketone compound of a heavy metal in a liquid hydrocarbon that is in physical contact with water, said compound being susceptible to hydrolysis or hydration, which method comprises increasing the hydrogen ion concentration of the 60 water present to a point at which hydrolysis and hydration of said compound is inhibited by the addition to said water of a hydrogen ion furnishing substance relatively insoluble in said hydrocarbon.

6. The method of stabilizing a solution of a beta diketone compound of a heavy metal in a liquid hydrocarbon that is in physical contact with water, said compound being susceptible to hydrolysis or hydration, which method comprises 70 increasing the hydrogen ion concentration of the water present to a point at which hydrolysis and hydration of said compound is inhibited by the addition of boric acid to said water.

7. The method of stabilizing a solution of a 75

beta diketone compound of a heavy metal in a liquid hydrocarbon that is in physical contact with water, said compound being susceptible to hydrolysis or hydration, which method comprises increasing the hydrogen ion concentration of the water present to a point at which hydrolysis and hydration of said compound is inhibited by the addition of phosphoric acid to said water.

8. The method of stabilizing a solution of a beta diketone compound of a heavy metal in a liquid hydrocarbon that is in physical contact with water, said compound being susceptible to hydrolysis or hydration, which method comprises increasing the hydrogen ion concentration of the water present to a point at which hydrolysis and hydration of said compound is inhibited by the addition of lactic acid to said water.

9. A stabilized storage system of a liquid hydrocarbon motor fuel containing a heavy metal beta diketone compound having a tendency to precipitate therefrom in the presence of water, said system comprising a liquid hydrocarbon

phase containing a heavy metal beta diketone compound dissolved therein, and a relatively immiscible aqueous phase in direct contact with said first phase having dissolved therein an acid reacting substance insoluble in said first phase, said acid reacting substance furnishing solely by virtue of dissociation due to solution a sufficient stable hydrogen ion concentration at the interface between said phases to inhibit said tendency of said heavy metal organic compound to precipitate.

10. A stabilized storage system as defined in claim 9, wherein the acid reacting substance is boric acid.

11. A stabilized motor fuel system as defined by claim 9, wherein the acid reacting substance is phosphoric acid.

12. A stabilized motor fuel storage system wherein the acid reacting substance is lactic acid.

WILLARD E. LYONS.

5

10

15

20